

Jan. 23, 1923.

1,443,081

J. D. MACKINTOSH.  
SOCK FOR BOOTS AND SHOES.  
FILED DEC. 16, 1920.



INVENTOR  
John Dickens Mackintosh  
of Clowden & Brier  
atty  
5

## UNITED STATES PATENT OFFICE.

JOHN DICKENS MACKINTOSH, OF MANCHESTER, ENGLAND.

## SOCK FOR BOOTS AND SHOES.

Application filed December 16, 1920. Serial No. 431,176.

*To all whom it may concern:*

Be it known that I, JOHN DICKENS MACKINTOSH, a British subject, residing at Openshaw, city of Manchester, county of Lancashire, England, have invented certain new and useful Improvements in Socks for Boots and Shoes, of which the following is a specification.

This invention relates to improvements in socks or insoles for boots and shoes.

It consists essentially in treating a sock or insole constructed in the usual way of felt, wool, flannel, or the like, with capsaicin, (extract of capsicum) and methyl salicylate (oil of wintergreen).

The sock or insole A is prepared in the usual way of felt, wool, flannel, or the like with or without a stiffening piece of cardboard. The material before being made up into the form of a sock or insole or the sock or insole is dyed with chrysoidium yellow to give it a yellow or orange colour.

The sock or insole is then saturated with a solution of capsaicin made up as follows:

Capsaicin ----- 1 oz.  
Methylated spirit ----- 50 oz. fluid.  
Water ----- 29 oz. fluid.

The sock or insole is then dried in warm room or chamber and after drying is sprayed with a solution of oil of wintergreen (methyl salicylate) and castor oil in methylated spirit made up in the following proportions:

Oil of wintergreen----- 1 fluid oz.  
Castor oil----- 1 fluid oz.  
Methylated spirit ----- 8 fluid oz.

The addition of the castor oil prevents the oil of wintergreen volatilizing too readily.

After spraying with the oil of wintergreen solution is dried at a temperature of about 120° F., and finally pressed.

Instead of treating the sock after it has been made up the material may be first treated and then made into a sock.

A sock or insole so treated will have thermal properties and assist in keeping the feet of the wearer warm in cold weather.

What I claim as my invention and desire to protect by Letters Patent is:

1. An insole for boots or shoes impregnated with an extract of capsicum and oil of wintergreen (methyl salicylate) in an amount sufficient to produce a stimulant action without irritation.

2. The method of producing an insole having thermogenic properties consisting in saturating the insole with a solution of capsaicin in methylated spirit, drying, spraying with a solution of methyl salicylate and finally drying and pressing.

In testimony whereof I have hereunto set my hand in presence of two subscribing witnesses.

JOHN DICKENS MACKINTOSH.

Witnesses:

J. OWDEN O'BRIEN,  
GEO. H. O'BRIEN.